

## 1

2,922,714

## COLUMBIUM-TANTALUM-ALUMINUM ALLOY

John L. Benham, Lewiston, N.Y., assignor to Union Carbide Corporation, a corporation of New York

No Drawing. Application April 3, 1957  
Serial No. 650,291

4 Claims. (Cl. 75—138)

This invention relates to a columbium-tantalum-aluminum alloy particularly adapted as an additive for titanium base alloys.

Titanium exists in either of two crystalline forms. At low temperatures, it exists in the hexagonal crystal form known as the alpha phase, and transforms at about 885° C. into the cubic crystal form known as the beta phase. Beta alloys are generally characterized by excellent weldability and are admirably suited in the production of titanium sheet alloy where bending properties are the criterion. However, some general disadvantages of the beta titanium base alloys are their poor tensile ductility, poor retention of strength at elevated temperatures, and poor metallurgical stability. On the other hand, alpha titanium base alloys are much more stable and possess good retention of strength at elevated temperatures and good tensile ductility. The chief disadvantage of the alpha type titanium alloy is its poor bend ductility. Because of the increasing use of titanium in industry, there is a demand for a titanium product having the beneficial properties of both the alpha and the beta titanium alloys.

Certain alloying additions to a titanium base metal, among which are columbium and tantalum, serve to increase the structural strength of titanium alloys. These constituents are usually added as pure metals or as ferro-alloys, such as ferrocolumbium or ferrotantalum-columbium. The addition of these desirable constituents as relatively pure metals is an expensive procedure and has the added disadvantage of poor rate of solution because of the high melting points of the pure metal additives. Both tantalum and columbium metals are highly malleable materials and, therefore, lack the requisite brittleness to be reduced to powder form. Tantalum and columbium additions as commercial alloys present a problem in controlling the introduction of such deleterious elements to titanium as oxygen, hydrogen, nitrogen, iron, carbon and silicon, which are normally present in ferrocolumbium and ferrotantalum-columbium in substantial percentages.

It is therefore an important object of the present invention to provide an addition agent for a titanium melt that is effective in producing a stable titanium base alloy having a desirable combination of good weldability, good tensile and bend ductility, the retention of strength at elevated temperatures, and a higher service temperature than present day all-alpha titanium base alloys.

Another object of the present invention is to provide an addition alloy of columbium-tantalum-aluminum which can be economically used as an addition agent for the production of a stable titanium base alloy.

Another object of the present invention is to provide an addition alloy of columbium-tantalum-aluminum essentially free of such deleterious elements to titanium as oxygen, nitrogen, hydrogen, iron, carbon and silicon.

Another object of the invention is to provide an addi-

## 2

tion alloy of columbium-tantalum-aluminum which can be readily reduced to finely divided form by means of conventional crusher apparatus.

The invention by means of which these objects are achieved is based on the discovery that the addition to a titanium melt of a properly proportioned master alloy, in which both alpha and beta phase promoters are present, produces an excellent grade of titanium alloy having an advantageous combination of desirable characteristics found in all-alpha titanium alloys and all-beta titanium alloys. The master alloy of the invention comprises as essential constituents, columbium and tantalum, which are known to retard the formation of alpha-phase titanium and to stabilize the beta phase titanium, and aluminum which has a strong tendency to promote the formation of alpha-phase titanium. Small amounts of other elements such as iron, silicon and manganese may be present in limited amounts, and gaseous impurities such as oxygen, hydrogen and nitrogen may be present as incidental impurities. The addition of the subject alloy results in a titanium alloy having a stable structure comprising an 'alpha matrix' in which some beta phase is present.

In a preferred embodiment of the alloy addition of the invention, the range of composition should be within the following limits.

|                       | Broad, percent | Preferred, percent |
|-----------------------|----------------|--------------------|
| Ta                    | 10-35          | 10-20              |
| Cb                    | 10-35          | 25-35              |
| Al                    | 20-75          | 35-55              |
| Fe                    | up to 3.0      | up to 2.5          |
| Si                    | up to 1.5      | up to 1.0          |
| Mn                    | up to 7.0      | up to 5.5          |
| O+H+N                 | up to 0.5      | up to 0.25         |
| Incidental impurities | remainder      | remainder          |

Optimum results are obtained within the above range when the ratio of columbium to tantalum is approximately 2 to 1, the ratio of aluminum to the combined tantalum and columbium content is 5 to 3, the iron does not exceed 4% of the combined tantalum and columbium content, the silicon does not exceed 1.5% of the tantalum and columbium, and the total oxygen, hydrogen and nitrogen not exceeding 0.5% of the tantalum and columbium.

In Table I are set forth results obtained on analysis of a typical addition alloy of the invention. The typical alloy addition was made in a heat in which fused columbium-tantalite and crude columbium oxide of the following compositions were reduced with excess aluminum in the presence of lime to produce a tantalum-columbium alloy containing 50% Al.

|                                | Fused Columbium-tantalite | Columbium Oxide |
|--------------------------------|---------------------------|-----------------|
| Ch <sub>3</sub> O <sub>5</sub> | 34.06                     | 86.39           |
| Ta <sub>2</sub> O <sub>5</sub> | 35.05                     | 1.28            |
| TiO <sub>2</sub>               | 1.18                      | 10.02           |
| Fe <sub>2</sub> O <sub>3</sub> | 2.60                      | 0.80            |
| MnO                            | 11.08                     | —               |
| SnO <sub>2</sub>               | 0.02                      | —               |
| SiO <sub>2</sub>               | 1.08                      | 0.12            |
| C                              | 0.01                      | —               |

The materials were melted in an electric arc furnace and thereafter tapped to produce a specimen of the following composition.

**3**  
**TABLE I**  
*Chemical analysis*

| Element:   | Percent   |
|------------|-----------|
| Cb         | 27.76     |
| Ta         | 12.82     |
| Al         | 49.85     |
| Ti         | 1.79      |
| Fe         | 1.45      |
| Si         | 0.54      |
| Mn         | 4.75      |
| C          | 0.05      |
| N          | 0.014     |
| O          | 0.010     |
| H          | 0.013     |
| Impurities | Remainder |

As a feature of the invention, the subject alloy possesses good crushability, an important attribute which is economically desirable in alloy additions, particularly those containing tantalum and columbium constituents. Shown in Table II below are the results of a typical screen analysis of the alloy specified in Table I. The alloy was readily crushed in conventional crusher apparatus.

**TABLE II**  
*Screen analysis*

| Retained on:  | Percent |
|---------------|---------|
| 1/4"          | Nil     |
| 8 Mesh        | 88.88   |
| 20 mesh       | 8.03    |
| 48 mesh       | 1.41    |
| 100 mesh      | 0.94    |
| Thru 100 mesh | Balance |

From the above it will be seen that the columbium-tantalum-aluminum alloy embodied in the present invention possesses favorable pulverulent properties, being readily reducible to powder form.

The following Table III indicates the importance of the use of a typical addition alloy of the invention in the production of a final titanium base alloy having 8% aluminum, 2% columbium, 1% tantalum, the balance iron, titanium and incidental impurities. Typical properties of this final titanium base alloy are tabulated as follows:

**TABLE III**

| <i>Typical mechanical properties of annealed Ti base alloy sheet (.040" thick)</i> |                 |
|------------------------------------------------------------------------------------|-----------------|
|                                                                                    | .040 inch sheet |
| Ultimate tensile strength (p.s.i.)                                                 | 127,000         |
| Yield Strength, 0.2% offset (p.s.i.)                                               | 120,000         |
| Elongation (percent)                                                               | 16              |
| Min. bend radius ( $\frac{\text{bend radius}}{\text{thickness}}$ )                 | 3-4             |

**4**

Welding tests on the above final titanium base alloy indicated that the alloy is readily welded with the same techniques used for commercially pure titanium, and that the weld sections possess substantially the same bend ductility and mechanical properties as the unwelded sections of the alloy.

From the above it will be seen that the tantalum-columbium-aluminum master alloy of the present invention is ideally suited as an addition agent to a titanium base alloy. When added to a titanium alloy, it is effective in producing a titanium base alloy having a highly desirable combination of properties previously occurring in part in alpha titanium alloys and beta titanium alloys. In addition, the alloy of the invention is easily reduced to powder form, and its use in readily prepared accurate quantities substantially reduces production costs.

It will be understood that modifications and variations may be effected without departing from the spirit and scope of the novel concepts of the present invention.

What is claimed is:

1. A columbium-tantalum-aluminum alloy consisting essentially of about 10% to 35% tantalum, 10% to 35% columbium, and the remainder aluminum and incidental impurities.
2. A columbium-tantalum-aluminum alloy consisting essentially of about 10% to 20% tantalum, 25% to 35% columbium, and the remainder aluminum and incidental impurities.
3. A columbium-tantalum-aluminum alloy consisting essentially of about 10% to 35% tantalum, 10% to 35% columbium, 20% to 75% aluminum, up to 3% iron, up to 1.5% silicon, up to 7% manganese, up to 0.5% of oxygen, hydrogen and nitrogen, and the remainder incidental impurities.
4. A columbium-tantalum-aluminum alloy consisting essentially of about 10% to 20% tantalum, 25% to 35% columbium, 35% to 55% aluminum, up to 2.5% iron, up to 1.0% silicon, up to 5.5% manganese, up to 0.25% oxygen, hydrogen and nitrogen, and the remainder incidental impurities.

45 **References Cited in the file of this patent**

**UNITED STATES PATENTS**

|           |               |               |
|-----------|---------------|---------------|
| 2,369,354 | Kempf et al.  | Feb. 13, 1945 |
| 2,579,369 | Dawe          | Dec. 18, 1951 |
| 2,711,960 | Methe         | June 28, 1955 |
| 2,740,711 | Herres et al. | Apr. 3, 1956  |
| 2,754,204 | Jaffee et al. | July 10, 1956 |
| 2,769,707 | Vordahl       | Nov. 6, 1956  |